

June 13, 1950

S. J. KOCH

2,511,164

PROCESS OF SEALING CONTACT TERMINALS TO ELECTRON TUBES

Original Filed May 2, 1945

*Fig. 1*



*Fig. 3*



*Fig. 2*



*Stanley J. Koch, INVENTOR.*

*BY  
Charles W. Mortimer*

## UNITED STATES PATENT OFFICE

2,511,164

## PROCESS OF SEALING CONTACT TERMINALS TO ELECTRON TUBES

Stanley J. Koch, Clifton, N. J., assignor to Allen B. Du Mont Laboratories, Inc., Passaic, N. J., a corporation of Delaware

Original application May 2, 1945, Serial No. 591,465. Divided and this application May 13, 1948, Serial No. 26,776

2 Claims. (Cl. 49—81)

1

This is a division of my application, Serial No. 591,465, filed May 2, 1945, which issued September 7, 1948, as Patent No. 2,448,808.

This invention relates to a process of securing a terminal or contact in the wall of a cathode-ray tube or electron tube for making connection from a source of electrical potential to an electrode extending inside of said tube.

Heretofore, connections of this type have been made by fusing a portion of the glass wall of the tube and locating the terminal so that a lead could be connected thereto. With such connections the glass tube was in danger of being broken or cracked by the contact being struck or too much pressure being applied thereto. Besides, since the contact surface between the contact member and the wall of the tube was not much more than was provided by the thickness of the wall of the tube, the danger of leaking and breaking the vacuum in the tube was increased.

By the present invention prior difficulties have been overcome and an electrical contact element is securely and firmly mounted on the tube in such a way that the danger of the tube being broken by force applied to the contact or a blow striking and breaking it is minimized, and at the same time the danger of leakage of air through the part where the contact is installed in the wall of the tube is materially decreased or entirely overcome.

The invention may be understood in connection with the accompanying drawing; in which:

Fig. 1 is a plan view of the contact;

Fig. 2 is a side view partly in section showing the contact and a pin therefor, which pin has a short cylinder of glass thereon; and

Fig. 3 is a sectional view showing a portion of the wall of a tube with the contact in place.

In the drawing, reference character 1 indicates the rounded portion or head of a contact to which connection is to be made from a source of potential. This connection may be made, for example, by a snap terminal which is held on head 1 in the known way.

Head 1 extends into a neck portion 2 which is flared outwardly into a disc portion 3 which is turned upwardly as indicated at 4 and ends in a downwardly extending ring portion, the end of which is shown by the reference character 5.

A metal rod 6 is installed in the neck portion 2 of the contact 1 and fits tightly therein so as

2

to maintain both a mechanical and electrical connection between the contact 1 and rod 6.

A glass bead 7 is placed on the rod 6 with one end thereof in contact with the portion 3 of the terminal.

A hole or opening slightly larger than the bead 7 is provided in a wall 8 of the tube where the contact is to be installed. The bead 7 and rod 6 are placed in this hole with the disc portion 10 of the contact 1 in contact with the outer surface of the glass wall. The glass is then fused by applying heat to it and the corresponding portion of the bead 7 to fuse the same together as shown in Fig. 3 and also to fuse the bead 7 more securely on the rod 6, and also fuse the glass so that it flows slightly around the portion 4 of the contact as indicated at 9, thus more securely anchoring the contact in the glass wall and also decreasing the danger of a leakage path 20 forming.

What is claimed is:

1. The process of sealing a contact terminal to the wall of an electron tube, which comprises forming a metal contact with a head and neck, 25 said neck terminating in an outwardly extending portion having an inwardly curved flange, locating an end of a metal rod in said neck, placing a glass tube on said rod, placing said outwardly extending portion of said neck on the outside wall 30 of said electron tube, fusing the wall of said electron tube where said contact terminal is located, fusing the wall of said glass tube to said curved flange and fusing one end of said glass tube to the wall of said electron tube.

2. The process of sealing a contact terminal to a wall of a glass tube, which consists in securing a metal rod to said terminal, placing a glass bead on said rod, providing a hole in the wall of said tube, inserting said rod and said glass bead into said hole, fusing said rod and said glass bead to said wall and said rod, and fusing said wall to a portion of said terminal.

STANLEY J. KOCH.

## REFERENCES CITED

The following references are of record in the file of this patent:

## UNITED STATES PATENTS

| Number    | Name     | Date          |
|-----------|----------|---------------|
| 2,089,044 | Thomas   | Aug. 3, 1937  |
| 2,151,809 | Shardlow | Mar. 28, 1939 |